

March 25, 1958

R. DE S. COUCH ET AL

2,828,240

PACKAGING MATERIAL

Filed Oct. 22, 1954



INVENTORS  
ROBERT DE S. COUCH  
MILTON YEZEK

BY  
Cameron, Kerkam & Sutton  
ATTORNEYS

1

2,828,240

## PACKAGING MATERIAL

Robert de S. Couch and Milton Yezek, Battle Creek, Mich., assignors to General Foods Corporation, White Plains, N. Y., a corporation of Delaware

Application October 22, 1954, Serial No. 464,169

12 Claims. (Cl. 154—138)

This invention relates to improved packaging material especially adapted for use in retail packaging or cartoning of goods that must be protected against loss of moisture to or absorption of moisture from outside the package.

Much time and attention have been devoted to the development of retail packages of the type characterized above. In general, such packages should have an attractive external dress and appearance, yet at the same time they should be highly resistant to the transfer of moisture or water vapor. As a rule, these requirements have been met by multiple packages in which printed cardboard cartons are the principal elements and protection against water vapor transfer (WVT) is increased by liners and/or single or double overwraps of foil, cellulosic films such as cellophane, glassine, waxed sulphite papers, and the like. But such arrangements are expensive, both as to material cost and as to the expense of inserting and/or overwrapping and then closing the successive layers of packaging material, with the result that desirable protection against water vapor transfer is often sacrificed in the interest of economy. As an illustration, breakfast cereals are commonly marketed today in printed cardboard cartons having single waxed and heat-sealed sulphite overwraps, although the WVT properties of such packages are no more than fair to begin with and deteriorate rapidly when the packages are jarred during handling.

Efforts have accordingly been made to provide by lamination a single sheet which will meet all of the aforementioned requirements and if possible provide improved WVT characteristics at the same time. For example, some degree of success has been attained by laminating two sheets of cardboard together with a moisture-resistant adhesive such as microcrystalline wax, but for good results the wax must be specially selected and/or modified so that it becomes tacky before too much can be absorbed by the board. Otherwise excessive quantities of laminant are absorbed with the results that the board may become so greasy that it can not be printed satisfactorily, and the amount of laminant remaining on the surface may be insufficient and too unevenly distributed to form a good bond. On the other hand, even though satisfactory lamination is obtained, the WVT properties obtained in this way do not provide the desired improvement over cartons with waxed paper overwraps as described above.

We have found that if the board is first impregnated as set forth hereinafter, it may then be laminated to paper

with substantial elimination of the difficulties set forth

above and production of an improved product as regards WVT properties. As a rule the impregnated board forms the inside of the carton or package and will be so considered hereinafter, although this is not necessarily the case. The other ply of the laminated product, which usually will be the outer ply of the package, may be no more than paper printed like the usual carton or overwrap. By virtue of the impregnation of the board ply, less laminant is required while a better bond is obtained, and notably superior WVT characteristics can be provided as set forth in detail below.

The board forming the inner ply of the laminated material may be any of a wide variety of known kinds: for example, boards made from pure chemical pulps such as bleached and unbleached kraft, soda and sulphite board; boards made from semi-chemical pulp such as corrugating medium board; and bleached semi-chemical board; board made from waste materials such as chip board and拒板 (rejute board); and board made from combinations of waste, groundwood, and chemical pulps such as White Patent coated news board, double Manila lined news, groundwood center, and double bleached lined waste-groundwood center board. Such board is normally specified in weight per thousand square feet and in points thickness (one point = 0.001 inch); on this basis any of the above types of board in the range of 20-160 lbs. and 5-40 point may be suitable for use depending upon the size of the package, the weight and physical form of the enclosed material, and the conditions to which the package is to be subjected.

The board selected for the inner ply is then impregnated before lamination. Generally speaking, any suitable impregnant can be employed which provides good WVT properties; examples are paraffin wax, microcrystalline waxes, polyethylene, asphalt, polyamides, and the like. By impregnated we mean not merely that the board is surface coated, but that the voids and interstices within the board are filled with the impregnant to a substantial depth below the surfaces of the board. A surface coating alone does not provide a satisfactory product. If made thick enough to provide in effect another ply of the coating material per se, the amount required is excessive; besides the coating material tends to be driven into the board unevenly during subsequent processing of the laminated structure, resulting in a tendency to delamination or at least weakened resistance to water vapor transfer at random points and thus in a non-uniform product. Thus the board should carry at least 10% by weight of impregnant, the major portion of which is impregnated into the material in the sense described above as distinguished from a surface coating. In fact, there need be no surface coating at all, although it is not necessary to take special pains to avoid it.

Preferably the board is treated under conditions such as pressure or vacuum which cause the impregnant to be driven thoroughly into the board. By such preferred methods board can be caused to absorb as much as 30-35% by weight of impregnant, the voids and interstices in the product being substantially all filled with im-

pregnant. For the types, weights and calipers of boards here involved, this condition of substantially full impregnation requires the absorption of at least 20% by weight of impregnant. As shown by the test results set forth hereinafter, such full impregnation prior to lamination results in outstandingly good WVT properties.

The other ply of the laminated material (usually but not necessarily the outer ply of the package) comprises a suitable paper, in most cases a paper capable of being printed, in the range of 8-90 lbs. (basis 24 x 36-500=3000 sq. ft.). Various kinds of paper are known, and as examples any of the following can be used: papers made from chemical pulps including sulphate papers, sulphite papers, sulphate-sulphite combination papers, and soda pulp papers, these various papers being either uncoated or coated on one or both sides with a coating comprising clay, titanium dioxide, and binder; papers made from chemical pulp or chemical pulp and groundwood combinations, coated or uncoated, which have been calendered or supercalendered such as publishing papers, glassine, supercalendered sulphite papers, machine finish sulphite-sulphate papers, and machine finish and machine glazed sulphite-sulphate papers; and other materials such as cellulosic films including cellophane and cellulose acetate, foil and the like.

The laminant is applied to one or both surfaces to be laminated and these surfaces are then juxtaposed in any suitable manner, with or without heat and/or pressure as may be appropriate to the particular impregnants and laminants involved. Various procedures and apparatus for laminating materials together are well known in the art and need not be set forth in detail. For quantity production, of course, it will be desirable to laminate strips or sheets running continuously over rolls, the laminant being applied by spraying, dipping or brushing as may be most convenient. Suitable laminants include, for example, microcrystalline waxes alone or with added polyethylene, butyl rubber, polyisobutylene, and/or paraffin; paraffin; polyethylene (2000-21,000 N. W.); vinyl acetate emulsions; polyamides; butyl rubber emulsions; and like moisture-proof adhesives.

The accompanying drawing illustrates diagrammatically one embodiment of the invention, but it is to be expressly understood that said drawing is by way of example only and is not to be taken as a definition of the limits of the invention, reference being had to the appended claims for this purpose.

In the drawing, the board which is to be impregnated and form the inner ply is drawn from any suitable supply, preferably in the form of a continuous web or strip 1, and passes through a suitable evacuated chamber 2 containing a bath 3 of hot liquid impregnant. The strip is caused to move through the bath by means such as the guide rollers 4, 5, and 6, dipping under the surface of the bath and then emerging from the bath before leaving the evacuated chamber.

Beyond the vacuum chamber, the desired moisture-resistant adhesive is applied to the strip and distributed over its surface by any suitable means as indicated by the arrow 7. Then while the moving strip with its impregnant and adhesive is kept hot by heating means 8 disposed along the path of travel, the paper that is to form the outer ply is drawn from any desired source, preferably in the form of a continuous web or strip 9 which passes around a roller 10 into a path parallel to that of the strip 1. The two strips 1 and 9 are then suitably pressed together, as by passing them between rollers 11, 12 completed, the laminated strip or web leaving the rolls at 12.

In the following tests, impregnated 8 pt. and 10 pt. bleached kraft board was laminated to a 60# paper coated on both sides with clay and binder or with clay, binder and titanium dioxide (basis 25 x 38-500; equivalent to 54.5# per 3000 sq. ft.). These kraft boards were impregnated with 143°-145° F. AMP paraffin by running a web of the board through a vacuum chamber immersed in

a bath of melted paraffin. One side of the board was then coated with Quaker State amber microcrystalline wax by means of a laboratory coating applicator, the temperature of the microwax being 210°-230° F. and the impregnated board being heated to 220° F. to slow the solidification of the microwax and produce a fiber-tearing bond between the board and paper. The paper ply was placed on the hot laminant and pressure applied by means of a rubber roller. For comparison plain (non-impregnated) board was laminated to the same coated paper in a similar manner except that the board was coated with microwax while cold and the board and applied paper heated for 15-20 seconds before pressing. Also some of the plain and impregnated board was double laminated by 15 coating it with microwax on the reverse side and laminating it to 30# printing sulphite.

TABLE #1

## 20 Analysis of board before and after impregnation

| 25 | Analysis                       | Results |             |        |             |
|----|--------------------------------|---------|-------------|--------|-------------|
|    |                                | 8 pt.   |             | 10 pt. |             |
|    |                                | Plain   | Impregnated | Plain  | Impregnated |
| 30 | Weight/M sq. ft. pounds        | 34.7    | 44.4        | 42.0   | 55.6        |
|    | Caliper inches                 | 0.0079  | 0.0079      | 0.010  | 0.010       |
|    | Stiffness-MD                   |         | 33          |        | 71          |
|    | (Taber)-CD                     |         | 20          |        | 44          |
|    | Total Wax/M sq. ft. pounds     |         | 9.7         |        | 13.6        |
|    | Percent Impregnation           |         | 21.8        |        | 24.5        |
|    | WVT-gms./100 sq. in./24 hours: |         |             |        |             |
|    | Flat                           |         | 2.1         |        | 1.2         |
| 35 | Fold <sup>1</sup> grams        |         | 5.5         |        | 3.0         |

<sup>1</sup> The fold used for WVT analysis consisted of creasing each sample four times. Two creases, one inch apart, ran in the machine direction; the other two were similar running in the cross direction of the board or perpendicular to the first two. One score in each direction was pre-broken 90° and the other two 180°.

TABLE #2

## 40 Analysis of 8 pt. single laminations

| 45 | Analysis                         | Results |             |
|----|----------------------------------|---------|-------------|
|    |                                  | Plain   | Impregnated |
|    |                                  |         |             |
| 50 | Weight/M sq. ft. lbs             | 57.7    | 66.2        |
|    | Caliper inches                   | 0.0113  | 0.0115      |
|    | Stiffness-MD                     | 85      | 100         |
|    | (Taber)-CD                       | 44      | 53          |
|    | Weight of Laminant/M sq. ft. lbs | 6.8     | 7.8         |
|    | WVT-gms./100 sq. in./24 hours:   |         |             |
| 55 | Flat gms.                        | 0.40    | 0.20        |
|    | Fold <sup>1</sup> gms.           | 3.30    | 1.80        |

<sup>1</sup> See Table #1.

TABLE #3

## 60 Analysis of 8 pt. double laminations

| 65 | Analysis                         | Results |             |
|----|----------------------------------|---------|-------------|
|    |                                  | Plain   | Impregnated |
|    |                                  |         |             |
| 70 | Weight/M sq. ft. lbs             | 60.0    | 79.2        |
|    | Caliper inches                   | 0.0140  | 0.0144      |
|    | Stiffness-MD                     | 132     | 110         |
|    | (Taber)-CD                       | 86      | 80          |
|    | Weight of Laminant/M sq. ft. lbs | 13.1    | 9.8         |
|    | WVT-gms./100 sq. in./24 hours:   |         |             |
|    | Flat gms.                        | 0.84    | 0.22        |
|    | Fold <sup>1</sup> gms.           | 1.20    | 0.35        |

<sup>1</sup> See Table #1.

TABLE #4

## Analysis of 10 pt. single laminations

| Analysis                          | Results |              |
|-----------------------------------|---------|--------------|
|                                   | Plain   | Impreg-nated |
| Weight/M sq. ft. ....             | lbs.    | 68.6         |
| Caliper.....                      | inches  | 0.0142       |
| Stiffness—MD.....                 |         | 156          |
| (Taber)—CD.....                   |         | 71           |
| Weight of Laminant/M sq. ft. .... | lbs.    | 8.6          |
| WVT—gms./100 sq. in./24 hours:    |         |              |
| Flat.....                         | gms.    | 0.20         |
| Fold.....                         | gms.    | 2.30         |
|                                   |         | 0.13         |
|                                   |         | 0.34         |

<sup>1</sup> See Table #1.

- (3) 1 oz. bleached kraft carton lined with waxed 25# sulphite and overwrapped with waxed 25# sulphite.  
 (4) 8 oz. chip board carton with waxed glassine liner and waxed 25# sulphite overwrap.  
 (5) 5½ oz. chip board carton with waxed laminated glassine liner and waxed 25# sulphite overwrap.  
 (6) 6 oz. chip board carton with waxed 25# sulphite liner and double overwrap of Reyseal 050 foil and waxed 25# sulphite.

Some of the cartons were packed in shipping cartons and subjected to drop tests (1 oz. size—6 drops of 48 inches; 8 oz. size—6 drops of 30 inches); thereafter all cartons were stored at 100° F. and approximately 80% R. H. and moisture analyses made from time to time with the following results:

TABLE #8  
Results of moisture analysis—1 oz. study unhandled

| Hours in Storage.....               | Percent Moisture Content After Various Hours in Storage |     |      |      |       |       |       |       |
|-------------------------------------|---------------------------------------------------------|-----|------|------|-------|-------|-------|-------|
|                                     | 22                                                      | 43  | 68   | 88   | 114   | 165   | 237   | 334   |
| Package Combination:                |                                                         |     |      |      |       |       |       |       |
| Impreg.+single lam.....             | 2.9                                                     | 3.7 | 4.2  | 4.7  | ..... | 6.7   | 6.3   | 10.2  |
| Plain+single lam.....               | 3.6                                                     | 3.7 | 5.2  | 4.1  | ..... | 7.1   | 6.8   | 9.9   |
| Impreg.+dbl. lam.....               | 2.3                                                     | 3.2 | 3.4  | 3.8  | ..... | 5.3   | 5.2   | 7.6   |
| Plain+dbl. lam.....                 | 2.9                                                     | 3.3 | 6.0  | 5.7  | 6.6   | 7.1   | ..... | 8.7   |
| Plain ctn.+OW <sup>1</sup> (a)..... | 5.8                                                     | 9.1 | 11.9 | 12.5 | 13.1  | ..... | ..... | ..... |
| Plain ctn.+OW (b).....              | 5.0                                                     | 5.8 | 6.8  | 7.1  | 8.4   | ..... | ..... | ..... |
| Plain ctn.+dbl. OW.....             | 3.6                                                     | 3.5 | 4.4  | 4.5  | ..... | 6.4   | 6.3   | 6.9   |
| Plain ctn.+liner+OW.....            | 3.1                                                     | 3.8 | 4.2  | 4.5  | ..... | 5.4   | 5.7   | 5.8   |

<sup>1</sup> Overwrap.TABLE #5  
Analysis of 10 pt. double laminations

| Analysis                          | Results |              |
|-----------------------------------|---------|--------------|
|                                   | Plain   | Impreg-nated |
| Weight/M sq. ft. ....             | lbs.    | 87.7         |
| Caliper.....                      | inches  | 0.0180       |
| Stiffness—MD.....                 |         | 251          |
| (Taber)—CD.....                   |         | 147          |
| Weight of Laminant/M sq. ft. .... | lbs.    | 14.4         |
| WVT—gms./100 sq. in./24 hours:    |         |              |
| Flat.....                         | gms.    | 0.32         |
| Fold.....                         | gms.    | 0.57         |
|                                   |         | 0.12         |
|                                   |         | 0.33         |

<sup>1</sup> See Table #1.

The 8 pt. laminated boards were used to prepare 1 oz. breakfast cereal cartons and the 10 pt. laminated boards were made into larger breakfast cereal cartons as follows:

TABLE #6

## Design and dimensions of cartons used in package study

| Carton     | Dimensions                | Design          | Overlap |
|------------|---------------------------|-----------------|---------|
| 1 oz.....  | 23/4" x 13 1/2" x 4"      | glued both ends | full.   |
| 8 oz.....  | 6 1/4" x 29 1/2" x 9 1/2" | do.....         | 3/4"    |
| 5½ oz..... | 5 1/4" x 19 1/2" x 7 1/4" | do.....         | full.   |
| 6 oz.....  | 5 1/4" x 17 1/2" x 7 1/4" | do.....         | full.   |

After filling with breakfast cereals, the above packages were heat sealed with microwax and their WVT properties compared with the following:

TABLE #7

- (1) 1 oz. bleached kraft carton overwrapped with waxed 25# sulphite (specimens a and b).  
 (2) 1 oz. bleached kraft carton double overwrapped with two sheets waxed 25# sulphite.

- (3) 1 oz. bleached kraft carton lined with waxed 25# sulphite and overwrapped with waxed 25# sulphite.  
 (4) 8 oz. chip board carton with waxed glassine liner and waxed 25# sulphite overwrap.

(5) 5½ oz. chip board carton with waxed laminated glassine liner and waxed 25# sulphite overwrap.

(6) 6 oz. chip board carton with waxed 25# sulphite liner and double overwrap of Reyseal 050 foil and waxed 25# sulphite.

Some of the cartons were packed in shipping cartons and subjected to drop tests (1 oz. size—6 drops of 48 inches; 8 oz. size—6 drops of 30 inches); thereafter all cartons were stored at 100° F. and approximately 80% R. H. and moisture analyses made from time to time with the following results:

TABLE #8  
Results of moisture analysis—1 oz. study unhandled

| Hours in Storage.....               | Percent Moisture Content After Various Hours in Storage |     |      |      |       |       |       |       |
|-------------------------------------|---------------------------------------------------------|-----|------|------|-------|-------|-------|-------|
|                                     | 22                                                      | 43  | 68   | 88   | 114   | 165   | 237   | 334   |
| Package Combination:                |                                                         |     |      |      |       |       |       |       |
| Impreg.+single lam.....             | 2.9                                                     | 3.7 | 4.2  | 4.7  | ..... | 6.7   | 6.3   | 10.2  |
| Plain+single lam.....               | 3.6                                                     | 3.7 | 5.2  | 4.1  | ..... | 7.1   | 6.8   | 9.9   |
| Impreg.+dbl. lam.....               | 2.3                                                     | 3.2 | 3.4  | 3.8  | ..... | 5.3   | 5.2   | 7.6   |
| Plain+dbl. lam.....                 | 2.9                                                     | 3.3 | 6.0  | 5.7  | 6.6   | 7.1   | ..... | 8.7   |
| Plain ctn.+OW <sup>1</sup> (a)..... | 5.8                                                     | 9.1 | 11.9 | 12.5 | 13.1  | ..... | ..... | ..... |
| Plain ctn.+OW (b).....              | 5.0                                                     | 5.8 | 6.8  | 7.1  | 8.4   | ..... | ..... | ..... |
| Plain ctn.+dbl. OW.....             | 3.6                                                     | 3.5 | 4.4  | 4.5  | ..... | 6.4   | 6.3   | 6.9   |
| Plain ctn.+liner+OW.....            | 3.1                                                     | 3.8 | 4.2  | 4.5  | ..... | 5.4   | 5.7   | 5.8   |

TABLE #9  
Results of moisture analysis—1 oz. study drop tested

| Hours in Storage.....    | Percent Moisture Content After Various Hours in Storage |     |     |     |       |       |       |       |
|--------------------------|---------------------------------------------------------|-----|-----|-----|-------|-------|-------|-------|
|                          | 22                                                      | 43  | 68  | 88  | 114   | 165   | 237   | 334   |
| Package Combination:     |                                                         |     |     |     |       |       |       |       |
| Impreg.+single lam.....  | 2.3                                                     | 3.0 | 4.7 | 4.3 | ..... | 5.8   | ..... | ..... |
| Plain+single lam.....    | 2.7                                                     | 3.2 | 4.2 | 5.0 | ..... | 6.2   | ..... | ..... |
| Impreg.+dbl. lam.....    | 2.4                                                     | 3.2 | 3.6 | 4.1 | ..... | 4.5   | ..... | ..... |
| Plain+dbl. lam.....      | 2.9                                                     | 4.1 | 7.8 | 7.5 | 6.3   | ..... | ..... | ..... |
| Plain ctn.+OW (b).....   | 5.4                                                     | 7.4 | 8.7 | 9.6 | 10.5  | ..... | ..... | ..... |
| Plain ctn.+dbl. OW.....  | 3.8                                                     | 4.4 | 4.4 | 5.3 | ..... | 6.2   | ..... | ..... |
| Plain ctn.+liner+OW..... | 3.2                                                     | 4.0 | 4.4 | 4.9 | ..... | 5.7   | ..... | ..... |

TABLE #10  
Results of moisture analysis—8 oz. study unhandled

| Hours in Storage.....    | Percent Moisture Content After Various Hours in Storage |     |     |     |      |       |       |       |
|--------------------------|---------------------------------------------------------|-----|-----|-----|------|-------|-------|-------|
|                          | 75                                                      | 123 | 219 | 316 | 366  | 556   | 756   | 1056  |
| Package Combinations:    |                                                         |     |     |     |      |       |       |       |
| Impreg.+single lam.....  | 3.5                                                     | 3.9 | 4.6 | 5.2 | 7.1  | 6.6   | ..... | ..... |
| Plain+single lam.....    | 3.8                                                     | 5.1 | 6.1 | 6.5 | 12.8 | 7.6   | ..... | ..... |
| Impreg.+dbl. lam.....    | 3.5                                                     | 4.6 | 4.1 | 5.3 | 7.2  | 7.3   | ..... | ..... |
| Plain+dbl. lam.....      | 3.7                                                     | 4.9 | 5.4 | 6.4 | 6.8  | 6.6   | ..... | ..... |
| Plain ctn.+liner+OW..... | 3.4                                                     | 3.8 | 4.4 | 4.9 | 5.9  | 7.3   | ..... | ..... |
| Plain ctn.+liner+OW..... | 3.5                                                     | 3.8 | 4.5 | 5.2 | 6.0  | ..... | ..... | ..... |

TABLE #11  
Results of moisture analysis—8 oz. study drop tested

| Hours in Storage.....    | Percent Moisture Content After Various Hours in Storage |     |     |     |     |     |       |       |
|--------------------------|---------------------------------------------------------|-----|-----|-----|-----|-----|-------|-------|
|                          | 75                                                      | 123 | 219 | 316 | 366 | 556 | 756   | 1056  |
| Package Combination:     |                                                         |     |     |     |     |     |       |       |
| Impreg.+single lam.....  | 3.9                                                     | 4.3 | 5.0 | 6.3 | 7.4 | 7.4 | ..... | ..... |
| Plain+single lam.....    | 4.0                                                     | 4.9 | 5.8 | 5.9 | 6.9 | 7.7 | ..... | ..... |
| Impreg.+dbl. lam.....    | 4.2                                                     | 4.5 | 5.0 | 5.6 | 6.8 | 5.8 | ..... | ..... |
| Plain+dbl. lam.....      | 3.9                                                     | 5.0 | 7.1 | 7.4 | 6.7 | 8.8 | ..... | ..... |
| Plain ctn.+liner+OW..... | 3.9                                                     | 4.9 | 5.8 | 6.0 | 7.6 | 7.2 | ..... | ..... |
| Plain ctn.+liner+OW..... | 4.3                                                     | 4.3 | 5.3 | 6.1 | 7.5 | 7.2 | ..... | ..... |

7  
TABLE #12

Results of moisture analysis—5 1/4 oz. study unhandled

| Hours in Storage.....    | Percent Moisture Content After Various Hours in Storage |     |     |     |     |
|--------------------------|---------------------------------------------------------|-----|-----|-----|-----|
|                          | 123                                                     | 221 | 385 | 551 | 624 |
| Package Combinations:    |                                                         |     |     |     |     |
| Impreg.+single lam.....  | 3.5                                                     | 4.0 | 4.9 | 5.9 | 6.1 |
| Plain ctn.+liner+OW..... | 2.2                                                     | 3.4 | 4.1 | 5.7 | 6.6 |

TABLE #13

Results of moisture analysis—6 oz. study unhandled

| Hours in Storage.....         | Percent Moisture Content After Various Hours in Storage |     |     |     |     |
|-------------------------------|---------------------------------------------------------|-----|-----|-----|-----|
|                               | 123                                                     | 221 | 385 | 551 | 624 |
| Package Combinations:         |                                                         |     |     |     |     |
| Impreg.+dbl. lam.....         | 1.8                                                     | 2.2 | 3.4 | 4.5 | 4.8 |
| Plain ctn.+liner+foil+OW..... | 1.6                                                     | 1.7 | 2.1 | 2.7 | 3.0 |

For purposes of comparison, it is convenient to find by interpolation in the above data the time required for the moisture content to increase from a given initial value to a selected final value. In considering breakfast cereals, it is appropriate to use for this purpose a range of 3.5–5.5% moisture corresponding generally to a critical range beyond which breakfast cereals tend to lose crispness noticeably.

In the above manner, taking 1-oz. package 1(b) of Table #7 as a standard of comparison, it is found that in all cases the laminated cartons provide superior moisture protection. Among the laminated structures, by far the best protection was afforded by those using paraffin-impregnated bleached kraft. The single laminated structure of this type was 50% better than the plain (non-impregnated) laminated structure and nearly 200% better than the standard. The double-laminated impregnated material was much better than the single-laminated impregnated material as would be expected.

Drop test handling had little or no effect on the laminated cartons, but resulted in marked decreases in the protection afforded by the unlaminated structures. Thus while special types of the latter having both waxed liners and waxed overwraps afforded very good protection before handling, they were no better than the single-laminated impregnated stock after drop testing. After handling, the latter provided approximately eight times better protection than the assumed standard.

Similar conditions were found with the larger cartons. In the 8-oz. and 5 1/4-oz. sizes the unhandled laminated-impregnated cartons were about equal to the plain carton having both liner and overwrap; after drop testing, however, the single-laminated impregnated carton was 10% better and the double-laminated impregnated material was 100% better. In the 6-oz. size, no drop tests were made.

Since commercially distributed packages are subjected to handling equivalent to that provided by the drop tests described above, it is evident that a fair evaluation of relative moisture protection can be obtained only after handling. The consistent marked superiority of the laminated-impregnated structures, as compared with both the laminated-non-impregnated structures and the cartons with separate liners and overwraps, is manifest from the foregoing data.

In another test designed to show that impregnation is not sufficient without lamination as well, the following results were obtained as an average of seven samples tested one per week for seven weeks:

8  
TABLE #14

Moisture pickup at 90° F. and 85% RH after 35 days storage

| Carton                                                                          | Moisture Pickup (Percent)                 |                                          |
|---------------------------------------------------------------------------------|-------------------------------------------|------------------------------------------|
|                                                                                 | Gelatin Dessert (Original Moisture 0.97%) | Starch Pudding (Original Moisture 3.16%) |
| 10                                                                              |                                           |                                          |
| Paraffin Impregnated Board.....                                                 | 10.25                                     | 6.12                                     |
| Paraffin Impregnated Board with Paraffin Coated Paper Overwrap.....             | 2.03                                      | 2.06                                     |
| 15 Paraffin Impregnated Board Laminated to Paper with Microcrystalline Wax..... | 0.59                                      | 1.06                                     |

From the foregoing data it is evident that the invention provides a new packaging or cartoning material offering marked advantages in the packaging of goods requiring protection against loss of moisture to or absorption of moisture from the outside atmosphere. In summary, these advantages reside in the fact that the single laminated sheet provides at least as good WVT properties as were obtainable heretofore with cardboard cartons and waxed paper overwraps, and especially in the further fact that these properties are not materially affected by handling of the packages whereas prior types of lined and overwrapped cartons rapidly lose a large if not major proportion of their original and intended WVT properties as the result of normal and unavoidable commercial handling. In addition, of course, the single laminated sheet is simpler and easier to handle than multiple prior cartons plus liners and/or overwraps, both in packaging the goods by the manufacturer and in opening the packages for use of the goods by the customer. At the same time there is no loss of attractiveness or adverse effect on the external dress or appearance of the packages, since as already indicated the outer paper ply may be printed in any desired manner. Thus by laminating a printed paper web to an impregnated board web, a laminated material is obtained that can be formed into cartons having the advantages set forth above together with elimination of liners and overwraps.

45 It is to be understood, of course, that the invention is not restricted to the details of the foregoing description and examples and that reference should be had to the appended claims for a definition of its limits.

What is claimed is:

- 50 1. A process for making laminated packaging material highly resistant to the transfer of water vapor therethrough which comprises impregnating board which is to form one ply by forcing a moisture-resistant impregnant amounting to at least 10% by weight of the board into the board under pressure so that the major portion thereof is absorbed by the board beneath its surface, juxtaposing a flat ply of said board and a second flat ply of paper, and laminating said previously impregnated board and paper together by interposing a moisture-resistant adhesive distributed over the juxtaposed flat faces of said plies and pressing the plies together.
- 55 2. The process defined in claim 1 in which the amount of said impregnant is from 20% to 35% by weight of the board.
- 60 3. A process for making laminated packaging material highly resistant to the transfer of water vapor therethrough which comprises juxtaposing two flat plies, one comprising 5–40 point board in the range of 20–160 lbs. weight per thousand square feet and previously impregnated with a moisture-resistant material amounting to at least 10% by weight of the board the major portion of which is absorbed into the board beneath its opposite surfaces, the other ply comprising paper in the range of 8–90 lbs. weight per three thousand square feet, coating the juxtaposed surface of one of said plies with
- 65
- 70
- 75

a moisture-resistant adhesive material distributed substantially uniformly over said surfaces, and pressing the plies together.

4. The process defined in claim 3, said impregnant being paraffinic wax and said adhesive being microcrystalline wax.

5. The process defined in claim 4, the amount of paraffinic wax being in the range of 20-35% by weight of the board.

6. The method of making laminated cartoning material which comprises forcing paraffin under pressure into a sheet of approximately 8-10 point kraft board with 20-35% by weight of paraffin to form one ply, juxtaposing a flat sheet of said board ply with a second flat ply comprising a sheet of printing paper of approximately 8-90 lbs. weight per three thousand square feet, interposing micro-crystalline wax as an adhesive between the paper and previously impregnated board, and distributed substantially uniformly over their juxtaposed flat surfaces and pressing them together while maintaining said paraffin in a molten condition during lamination.

7. A laminated packaging material comprising a ply of 5-40 point board in the range of 20-160 lbs. per thousand square feet in weight, said board being impregnated with a moisture-resistant impregnant amounting to at least 10% by weight of the board and the major portion thereof filling the voids in the board beneath its opposite surfaces, a second ply comprising paper in the range of 8-90 lbs. per three thousand square feet in weight, and a moisture-resistant laminating adhesive material interposed between said impregnated board ply and said paper ply, said plies being juxtaposed and adhesively united over their entire area by said interposed adhesive material.

8. A laminated packaging material comprising a ply of 5-40 point board in the range of 20-160 lbs. per thousand square feet in weight, said board being impregnated with a moisture-resistant impregnant amounting to at least 10% by weight of the board and the major portion thereof filling the voids in the board beneath its opposite surfaces, a second ply comprising paper in the range of 8-90 lbs. per three thousand square feet in

5

weight, said paper being printed on one side to form the external surface of a package, and a moisture-resistant laminating adhesive material interposed between said impregnated board ply and the other side of said paper ply, said plies being juxtaposed and adhesively united over their entire area by said interposed adhesive material.

9. A laminated packaging material as defined in claim 8, said impregnant comprising paraffinic wax.

10. A laminated packaging material as defined in claim 8, said adhesive material comprising microcrystalline wax.

11. A laminated packaging material as defined in claim 8, said impregnant being paraffin and said adhesive material being microcrystalline wax.

12. A laminated material for making moisture-resistant cartons comprising a ply of approximately 8-10 point kraft board impregnated with 20-35% by weight of paraffinic wax, the major portion of said impregnant filling the voids in the board beneath its opposite surfaces, a second ply of printing paper in the range of 8-90 lbs. weight per three thousand square feet, said plies being joined throughout substantially their entire area by interposed microcrystalline wax as an adhesive.

25

#### References Cited in the file of this patent

#### UNITED STATES PATENTS

|           |              |                |
|-----------|--------------|----------------|
| 395,645   | Anderson     | June 1, 1889   |
| 1,217,819 | Peterson     | Feb. 27, 1917  |
| 1,408,746 | Kick         | Mar. 7, 1922   |
| 1,618,491 | Taliaferro   | Feb. 22, 1927  |
| 2,158,754 | Hodgdon      | May 16, 1939   |
| 2,290,741 | Eckert       | July 21, 1942  |
| 2,296,171 | Magill       | Sept. 15, 1942 |
| 2,376,899 | Bulatkin     | May 29, 1945   |
| 2,434,106 | Flood et al. | Jan. 6, 1948   |
| 2,568,349 | McKee        | Sept. 18, 1951 |

30

35

|         |               |               |
|---------|---------------|---------------|
| 542,079 | France        | May 11, 1922  |
| 464,751 | Great Britain | Apr. 23, 1937 |

40

#### FOREIGN PATENTS

|               |               |
|---------------|---------------|
| France        | May 11, 1922  |
| Great Britain | Apr. 23, 1937 |